

1

3,549,358

**ELECTROPHOTOGRAPHIC PROCESS USING  
ORGANIC PHOTOCONDUCTORS HAVING  
AT LEAST TWO CHROMOPHORES**

Nicholas J. Clecak, San Jose, and Robert J. Cox, Los Gatos, Calif., assignors to International Business Machines Corporation, Armonk, N.Y., a corporation of New York  
No Drawing. Filed Dec. 23, 1968, Ser. No. 786,461  
Int. Cl. G03g 5/00

U.S. Cl. 96—1

2 Claims

**ABSTRACT OF THE DISCLOSURE**

The organic photoconductors are certain linear molecules having at least two chromophores such as a Schiff's base group or an azo group joined to one another through a benzene ring or series of benzene rings. These compounds have been found to be useful as photoconductors in electrophotographic processes. Some of the compounds are novel.

**BACKGROUND OF THE INVENTION**

**Field of the invention**

This invention relates to a class of organic photoconductive materials and, more particularly, relates to their use as photoconductors in electrophotographic processes, especially those utilizing contact reflex exposure.

**Description of prior art**

A number of organic photoconductors are known in the prior art, but most of them have not achieved commercial success because their sensitivity or exposure speed is too slow to compete favorably with the commercially used inorganic photoconductors, such as selenium. However, aside from speed, most organic photoconductors offer many advantages over the commercially used selenium. That is, photoconductive elements fabricated from organic photoconductors are easily manufactured, can be substantially translucent, and are sufficiently flexible to be used in belt configurations and the configurations of U.S. patent application Ser. No. 649,162 filed June 22, 1967, now abandoned.

U.S. patent application Ser. No. 668,697, filed Sept. 18, 1967, describes a contact reflex reproduction method. The compounds of the present invention are particularly useful in such a process.

U.S. patent applications Ser. No. 668,703, filed Sept. 18, 1967, now U.S. Pat. 3,489,558 and Ser. No. 668,696, filed Sept. 18, 1967, now U.S. Pat. 3,501,293 both describe other compounds useful as organic photoconductors.

**SUMMARY OF THE INVENTION**

It has now been found that a class of compounds offer the advantages of organic photoconductors, discussed above, and, in addition, exhibit dichroism. The compounds of the present invention are those having the formula:



wherein A is selected from the group consisting of



2



and



X is selected from the group consisting of:  $(-\text{CH}=\text{N}-)$ ,  $(-\text{N}=\text{CH}-)$ ,  $(-\text{N}=\text{N}-)$ ,  $(-\text{CH}=\text{CH}-\text{CH}=\text{N}-)$ , and  $(-\text{N}=\text{CH}-\text{CH}=\text{CH}-)$ ; and R is selected from the group consisting of hydrogen, nitro, lower dialkyl-amino, and lower dialkyl-aminophenylazo.

Of the compounds covered by the above general formula, the most preferred ones are those in which R is lower dialkyl-aminophenylazo while X is  $(-\text{CH}=\text{N}-)$  and A is



and also those in which R is lower dialkyl-amino while X is  $(-\text{CH}=\text{CH}-\text{CH}=\text{N}-)$  and A is



Both of these two classes of most preferred compounds are novel.

For the preparation of photoconductive elements, it is advantageous for the compounds of the general formula to be dissolved in organic solvents, such as tetrahydrofuran, or any other solvent in which the compounds are at least partially soluble. Such solutions are applied to substrates suitable for electrophotography and the solvent is then removed. Mixtures of solvents can also be used.

Instead of the above preparation, the compounds of the general formula can be used in conjunction with a resinous binder. Suitable resins include both natural and synthetic resins, examples of which are balsam resins, phenol resins modified with colophony, coumarone resins, indene resins, cellulose ethers, polyvinylchlorides, polyvinylacetate, acrylic polymers, such as polymethyl acrylic esters, polystyrene, polyisobutylene, polyvinylnormal, polycondensates, such as phthalate resins, polyamides, and polyadducts, such as polyurethanes.

The proportion of resin to the photoconductive compound can vary greatly, but elements having a high proportion of resin and a low proportion of photoconductive compound are the less desired. Mixtures of at least equal parts resin and photoconductive compound are preferred.

The substrate material, if one is desired, may be any which satisfy the requirements of electrophotography such as metal, glass, paper, or plastic. Unless it is to be used in a device employing dual corona discharge, such as U.S. Pat. 2,922,883, the substrate should preferably have a conductivity greater than  $10^{-10} \text{ ohm}^{-1} \text{ cm.}^{-1}$

Application of the solutions of the compounds of the general class, with or without resins, is in the usual manner, such as by spraying, doctor blade, meniscus coating, etc., followed by drying.

One type of electrophotographic process in which the compounds of the present invention are useful is known as xerography. The process comprises the laying down of the uniform electrostatic charge on a photoconductive insulating element, exposing the electrostatic charge surface to a pattern of light to effect a decay of charge in illuminated areas, and contacting the latent electrostatic image thus formed with colored electroscopic powder to render the image visible. Next, a copy sheet is brought into contact with the developed image and transferred thereto and fixed thereon. The residual toner remaining

on the photoconductive insulating element is removed by cleaning and the element is then ready for the preparation of the next copy or the next cycle.

Because they have the additional advantage of being dichroic, the compounds of the present invention are suitable for use in that type of electrophotography known as contact reflex reproduction, which is an electrophotographic process for the production of re-

flex copies in which a document is positioned adjacent a photoconductive element which exhibits photoconductive dichroism and has a preferred absorption axis, and in which the photoconductive element is uniformly exposed through the photoconductive element with polarized light whose vector, relative to the absorption axis, is such that the light is not absorbed. The polarized light in striking the document is absorbed in some areas, nor-



mally the dark image areas, and depolarized and reflected in others, normally the light background areas. The light from the reflected areas, being depolarized, contains light with an electric vector which will be absorbed by the photoconductive element and the element is thus exposed to a pattern corresponding to the pattern of the document. This renders the photoconductive element conductive and capable of transporting an electrostatic charge,



and, hence, permits the formation of an electrostatic charge pattern corresponding to the document.

The general nature of the invention having been set forth, the following examples are now presented as to the specific preparation of compounds falling within the above general class and the specific preparation of these compounds into photoconductive elements which are then used in electrophotographic processes. The specific details presented are for purposes of illustration and not limitation.

A general method for the preparation of the Schiff's base type of condensation product is as follows:

The difunctional aldehyde or diamine is dissolved in an alcohol such as n-butanol with a slight excess of the mono functional aldehyde or amine and heated to reflux for ½-2 hours. The resultant condensation products precipitate out of the hot reaction solvent and are hot filtered. They are subsequently washed with acetone, ether, and dried.

### EXAMPLE I

N,N' bis(p-dimethylaminobenzylidene) p-phenylene-diamine

$(\text{CH}_3)_2\text{N}-\text{C}_6\text{H}_4-\text{CH}=\text{N}-\text{C}_6\text{H}_4-\text{N}=\text{CH}-\text{C}_6\text{H}_4-\text{N}(\text{CH}_3)_2$

This compound was prepared by the above general method by refluxing in ethanol for one hour. It was iso-

70

lated as a yellow crystalline solid as shown in Beil., 14, 35. It had the following analysis.

Calcd. for  $\text{C}_{24}\text{H}_{26}\text{N}_4$  (percent): C, 77.8; H, 7.1; N, 15.1. Found (percent): C, 77.9; H, 7.1; N, 15.1.

### EXAMPLE II

1,4 bis benzylidene bis N,N dimethyl-p-phenylene-diamine



Prepared according to the general procedure by refluxing terephthaldehyde and N,N-dimethyl-p-phenylenediamine in ethanol for one hour. Isolated as an orange solid.

Calcd. for  $\text{C}_{24}\text{H}_{26}\text{N}_4$  (percent): C, 77.8; H, 7.1; N, 15.1. Found (percent): C, 78.3; H, 7.1; N, 14.5.

### EXAMPLE III

4,4' bis(p-dimethylaminobenzylideneamino) stilbene



Prepared following the general procedure by refluxing 4,4' diaminostilbene and p-dimethylaminobenzaldehyde for one hour in n-butanol. It was isolated as orange crystals as shown in Beil., 14 (I), 361.

Calcd. for  $\text{C}_{32}\text{H}_{32}\text{N}_4$  (percent): C, 81.3; H, 6.8; N, 11.8. Found (percent): C, 81.2; H, 6.8; N, 11.7.

### EXAMPLE IV

4,4' bis(p-dimethylaminobenzylideneamino) bibenzyl



Prepared by the general procedure using n-butanol and refluxing 4,4' diaminobibenzyl and p-dimethylaminobenzaldehyde for two hours. Isolated as yellow solids.

Calcd. for  $\text{C}_{32}\text{H}_{34}\text{N}_4$  (percent): C, 81.0; H, 7.2; N, 11.8. Found (percent): C, 81.1; H, 7.3; N, 11.7.

### EXAMPLE V

N,N' bis(benzylidene) benzidine



Prepared by the general procedure by refluxing benzidine and benzaldehyde in ethanol for ¼ hour as referenced in CA., 53:414 (1959).

Calcd. for  $\text{C}_{26}\text{H}_{20}\text{N}_2$  (percent): C, 86.6; H, 5.5; N, 7.8. Found (percent): C, 86.0; H, 5.5; N, 8.1.

### EXAMPLE VI

N,N' bis (p-dimethylaminobenzylidene) benzidine



Prepared by the general procedure by heating benzidine and p-dimethylaminobenzaldehyde in ethanol for one hour. Isolated as a yellow solid as shown in CA., 52:5197 (1958).

Calcd. for  $\text{C}_{30}\text{H}_{30}\text{N}_4$  (percent): C, 80.7; H, 6.8; N, 12.5. Found (percent): C, 80.8; H, 6.9; N, 12.4.

### EXAMPLE VII

N,N' bis (9-julolidinidene) benzidine



## 5

Prepared by the general procedure refluxing 9-formyljulolidene and benzidine in n-butanol for two hours. Isolated as yellow solids.

Calcd. for  $C_{38}H_{38}N_4$  (percent): C, 82.8; H, 6.9; N, 10.2. Found (percent): C, 82.7; H, 6.9; N, 10.3.

This compound fits into the general formula given above when the lower dialkyl-amino group R is considered to be linked at both ends to the phenyl ring.

## EXAMPLE VIII

N,N' bis (p-dimethylaminophenylazobenzilidene) benzidine



Prepared by the general procedure by refluxing benzidine and p-dimethylaminophenylazobenzaldehyde in ethanol for  $\frac{1}{4}$  hour. Isolated as red crystals.

Calcd. for  $C_{42}H_{38}N_8$  (percent): C, 77.0; H, 5.8; N, 17.1. Found (percent): C, 76.1; H, 5.9; N, 16.9.

This novel compound was found to be dichroic to an outstanding degree.

## EXAMPLE IX

N,N' (p-dimethylaminocinnamalidene) benzidine



Prepared by the general procedure by refluxing benzidine and p-dimethylaminocinnamaldehyde in ethanol for  $\frac{3}{4}$  hour. It was isolated as a brown solid.

Calcd. for  $C_{34}H_{34}N_4$  (percent): C, 80.2; H, 6.9; N, 11.2. Found (percent): C, 80.3; H, 6.9; N, 11.6.

## EXAMPLE X

4,4'-bis (p-dimethylaminophenylazo) biphenyl



This was prepared by diazotizing benzidine and coupling with dimethyl amiline as outlined in Aust. J. Chem., 1455 (1967).

## EXAMPLE XI

4,4' (bis p-nitrocinnamylidene) benzidine



0.45 g. benzidine and 1.5 g. p-nitrocinnamaldehyde in 100 ml. n-butanol were refluxed for 1 hour. The resulting precipitate was hot filtered and washed with acetone, ether and dried. Recovered 1.05 g. red colored solids.

Calcd. for  $C_{30}H_{22}N_4O_4$  (percent): C, 71.7; H, 4.4; N, 11.2. Found (percent): C, 71.8; H, 4.5; N, 11.4.

## EXAMPLE XII

Bis (p-dimethylaminophenylimino) bis 1,4-phenylene-2-propenylidene



Bis 1,4-phenylenepropenal and N,N-dimethyl-p-phenylenediamine are refluxed in ethanol. The resultant precipitate is hot filtered and the product worked up in a manner analogous to the above examples.

## EXAMPLE XIII

4,4' bis (p-dimethylaminocinnamylideneamino) stilbene



## 6

1 g. 4,4' diaminostilbene and 3 g. p-N,N-dimethylaminocinnamaldehyde in 150 ml. n-butanol were refluxed for 45 minutes. The resulting precipitate was hot filtered and washed with acetone, ether and dried. Recovered 0.75 g. brown solids. The product had the following analysis.

Calcd. for  $C_{32}H_{36}N_4$  (percent): C, 82.4; H, 6.9; N, 10.7. Found (percent): C, 81.6; H, 6.8; N, 10.9.

This novel compound was found to be very highly dichroic.

## EXAMPLE XIV

A photoconductive element was prepared by dispersing N,N' bis(p-dimethylaminobenzylidene)p-phenylenedi-

amine (the compound prepared in Example I above) in an equal weight of polystyrene dissolved in 1,2-dichloroethane and coating the solution on an aluminum slide with a doctor blade set at a 5 mil wet gap. The thus prepared photoconductive element was uniformly electrostatically charged using a Xerox Model D Processor at a potential of +7000 volts. After charging, the element was exposed to a 375 watt GE Photo EBR lamp at a distance of 12 inches for 2 seconds and using positive transparency as a document to be copied. The formed elec-

trostatic image was developed with negatively charged toner (Xerox 914) across the photoconductive element. Again using the Xerox Model D Processor, the toner image was transferred to paper by spraying positive charges on the back of the paper. After transfer of the toner image, the toner was fused to the paper on a hot



plate to yield a high quality copy of the document with high contrast, high image density, and faint background.

## EXAMPLE XV

A photoconductive element was prepared by dispersing N,N' bis(p-dimethylaminophenylazobenzilidene)ben-



zidine (the compound of Example VIII above) in an equal weight of polystyrene dissolved in 1,2-dichloroethane and coating the solution on an aluminum slide with a doctor blade set at a 5 mil wet gap. The thus prepared photoconductive element was uniformly electrostatically charged using a Xerox Model D Processor at a potential of +7000 volts. After charging, the element was exposed to a 375 watt GE Photo EBR lamp at a distance of 12 inches for 0.1 second and using positive transparency as a document to be copied. The formed electrostatic

image was developed with negatively charged toner (Xerox 914) across the photoconductive element. Again using the Xerox Model D Processor, the toner image was transferred to paper by spraying positive charges on the back of the paper. After transfer of the toner image, the toner was fused to the paper on a hot plate



to yield a high quality copy of the document with high contrast, high image density, and faint background.

## EXAMPLE XVI

Aluminized cellulose acetate is coated by means of a meniscus coater with 4% of a copolymer of methyl vinyl ether and maleic anhydride in water. The film is allowed to air dry overnight.

4,4'-bis(p-dimethylaminocinnamylideneamino) stilbene (the novel dichroic compound of Example XIII above) is applied to the above film by hand application in a linear direction along the length of the web. On top of this there is coated the following formulation:

|                                                                                                                             |       |
|-----------------------------------------------------------------------------------------------------------------------------|-------|
| 10% polyvinyl carbazole in benzene                                                                                          | G. 40 |
| Benzene                                                                                                                     | 20    |
| Chloroform                                                                                                                  | 30    |
| Toluene                                                                                                                     | 10    |
| 1,3-dinitronaphthalene                                                                                                      | 0.04  |
| 1% benzene solution of a plasticizer consisting of a combination of polymers of esters of acrylic acid and methacrylic acid | 8     |

This formulation is coated at 3 feet per minute on a meniscus coater and cured for 1 hour at 90° C. Electrometer results show a charge acceptance of about 600 v. The film is used to make robot copies in the contact reflex mode.

While the invention has been shown and described with reference to preferred embodiments thereof, it will be appreciated by those skilled in the art that variations in form may be made therein without departing from the spirit and scope of the invention.

What is claimed is:

1. In an electrophotographic reproduction process which comprises selectively rendering portions of a photoconductor electrically conductive by selective exposure to light, the improvement according to which the photoconductive element comprises a compound selected from the group consisting of compounds having the formula:



wherein A is selected from the group consisting of



and



X is selected from the group consisting of:



and  $(\text{--N}=\text{CH--CH}=\text{CH}\text{--})$ ; and R is selected from the group consisting of hydrogen, nitro, lower dialkylamino, and lower dialkyl-aminophenylazo.

2. A step of exposing the photoconductive element as claimed in claim 1 wherein the process is carried out in the contact reflex mode.

## References Cited

## UNITED STATES PATENTS

|           |         |             |      |
|-----------|---------|-------------|------|
| 3,066,023 | 11/1962 | Schlesinger | 96—1 |
| 3,163,532 | 12/1964 | Schlesinger | 96—1 |
| 3,335,003 | 8/1967  | Snelling    | 96—1 |
| 3,489,558 | 1/1970  | Cleak       | 96—1 |

GEORGE F. LESMES, Primary Examiner

M. B. WITTENBERG, Assistant Examiner

U.S. CL. X.R.

96—1.5, 252—501, 260—144, 576